

## UNITED STATES PATENT OFFICE

2,270,026

CATALYTIC TREATMENT IN STAINLESS  
STEEL APPARATUS

Robert P. Russell, Millburn, N. J., assignor to  
Standard Oil Development Company, a cor-  
poration of Delaware

No Drawing. Application August 19, 1939,  
Serial No. 291,041

2 Claims. (Cl. 196—133)

This invention relates to iron alloys of the type known as 25-20 stainless steel, and is more particularly concerned with an improved alloy of this type which is especially resistant to attack by carbon oxides.

Stainless steels of the 25-20 type contain from 24 to 26% chromium, 19 to 21% nickel and the balance iron and small amounts, usually less than 1%, of silicon, phosphorus, manganese and carbon. These steels are used extensively in processes for treating hydrocarbon oils at high temperatures and in the presence of hydrogen or other gases. Processes of this type are cracking, reforming, catalytic cracking, catalytic reforming and catalytic reforming in the presence of hydrogen.

In catalytic cracking a hydrocarbon oil such as a gas oil is passed at a temperature of 700 to 850° F. and under atmospheric or slightly elevated pressure over a catalyst such as Super-Filtrol, natural or activated clays of the bentonitic or montmorillonitic type, aluminum silicate, silica gel and the like, for the purpose of producing motor fuel of increased octane number.

In catalytic reforming a hydrocarbon oil consisting essentially of hydrocarbons boiling substantially in the gasoline range is passed at a temperature between 850° and 1050° F. under atmospheric or slightly elevated pressure and at a rate between 0.3 and 5.0 volumes of liquid oil per volume of catalyst per hour over a catalyst comprising a carrier or support such as alumina, silica gel, etc. and an active oxide of a metal of the IV, V, VI or VIII groups of the periodic system, for the principal purpose of increasing the octane number of the hydrocarbon oil without causing extensive reduction in molecular weight or boiling point. Among the reactions which occur in catalytic reforming to a greater or lesser extent depending upon the character of the feed, the type of catalyst and the operating conditions are dehydrogenation, aromatization or cyclization, desulfurization, isomerization and alkylation.

In catalytic reforming in the presence of hydrogen a hydrocarbon oil comprising hydrocarbons boiling substantially in the gasoline range is passed over a catalyst together with substantial quantities of hydrogen or a gas rich in free hydrogen at a temperature between 850 and 1050° F., under a pressure between 50 and 500 lbs. per square inch, and at a rate between 0.3 and 5.0 volumes of liquid oil per volume of catalyst per hour. The reason for using hydrogen will be apparent from what follows:

In all these catalytic processes the activity of the catalyst for promoting the reactions desired is gradually destroyed because of the deposition or formation on the catalyst of carbonaceous contaminants such as coke. It is then necessary to regenerate the activity of the catalyst and this is usually done by passing a mixture of hot inert gases and regulated quantities of air or oxygen therethrough whereby the coke and carbonaceous materials are removed by combustion. The flow of gases is ordinarily continued until no more oxygen is consumed. This indicates that most if not all of the coke has been burned off. The length of time that the catalyst can be used before requiring regeneration will depend upon how long the product produced meets the desired specifications. This time will vary from as little as 30 seconds in the case of catalytic cracking to as long as 6 to 12 hours or more in the case of catalytic reforming in the presence of hydrogen. It is of course desirable to be able to use the catalyst as long as possible before it requires regeneration and it has been found that by conducting the catalytic process in the presence of substantial quantities of added or recirculated hydrogen the tendency for coke deposition on the catalyst is greatly retarded and at the same time the quality of the product is still further increased.

During the regeneration of the catalysts used in these processes the coke is removed by combustion. Thus large quantities of carbon monoxide and carbon dioxide are formed. The temperatures during regeneration are ordinarily between 650 and 900° F. but spot temperatures as high as 1200° F. may be encountered. Under these conditions, definite though relatively minute quantities of iron carbonyl are formed by interaction of the iron in the steel parts of the apparatus and the carbon oxide evolved in the combustion.

Nearly all catalysts used in these catalytic processes are sensitive to and poisoned by minute traces of iron in certain forms. It is found that the iron carbonyl formed during regeneration of the catalysts subsequently decomposes and deposits traces of iron on the catalyst, thus poisoning it and causing a more or less permanent loss in activity which is not restored by regeneration.

The present invention has for its principal object a method of avoiding the formation of iron carbonyl during regeneration and the subsequent poisoning of the catalyst by the deposition of iron thereon.

I have found that by incorporating small quantities of silver in the 25-20 stainless steel used for the construction of reactors and tubing for catalytic processes of the type described, the tendency for the formation of iron carbonyl or at any rate for the deposition of minute traces of iron on the catalyst is substantially retarded or altogether prevented.

The quantity of silver added to the stainless steel alloy is in general below about 2%, and in most cases from 0.20 to 1.80% silver is sufficient. Thus a typical alloy would have a composition of 24% chromium, 19% nickel, 1.2% silver, and the balance iron and small amounts of carbon, silicon, phosphorus and manganese which do not interfere with the effect of the silver on the steel.

This silver containing stainless steel may be used for the construction of the entire apparatus or it may be used merely for the lining of those parts of the apparatus which come into contact with hot gases containing carbon monoxide. Ordinarily the reaction vessels used for catalytic processes of the type described have an inner lining of the 25-20 stainless steel and the outside is constructed of ordinary steel. In these cases the inner lining only need be made of the silver containing steel.

By using these silver alloys in catalytic reforming in the presence of hydrogen in place of the 25-20 stainless steel without the silver I have found that the activity of catalysts comprising activated alumina and chromium oxide or molybdenum oxide can be brought back by regeneration to substantially the initial activity of the fresh catalyst. In nearly every case previously it has been observed that after even the first regeneration the catalyst is not restored to its original activity and after each regeneration the activity is brought back to a progressively lower level. When using the silver 25-20 stainless steel alloy I have found that this progressive decrease in post-regeneration activity is greatly retarded.

It will be understood that while this silver alloy has been described as being of particular value in catalytic processes for treating hydrocarbon oils, it is of equal value in any process in which the formation of iron carbonyl and its subsequent decomposition may have deleterious effects.

This invention is not limited by any theories of the mechanism of the reactions nor by any details which have been given merely for purposes of illustration but is limited only in and by the following claims in which it is intended to claim all novelty inherent in the invention.

I claim:

1. In the catalytic treatment of hydrocarbon oils in apparatus constructed of the 25 chromium-20 nickel type stainless steel and in the presence of a catalyst which requires periodic regeneration to restore its activity, said regeneration being effected by burning off the coke deposited on the catalyst by passing hot gases containing oxygen therethrough, the method of preventing the formation of iron carbonyl by interaction of carbon monoxide formed in the regeneration with the iron of the steel alloy which comprises constructing those portions of the apparatus exposed to the hot gases during regeneration of steel containing from 24 to 26% chromium, 19 to 21% nickel, between 0.2 and 2% of silver and the balance iron and small amounts of carbon and other elements which do not interfere with the effect of the silver on the steel.

2. In catalytic reforming in the presence of hydrogen carried out in apparatus constructed of or lined with the 25 chromium-20 nickel type of stainless steel and in the presence of a catalyst which requires periodic regeneration to restore its activity, said regeneration being effected by burning off the coke deposited on the catalyst by passing hot inert gases containing oxygen therethrough at a temperature between 650 and 1200° F., the method of preventing the formation of iron carbonyl by interaction of the carbon monoxide evolved in the regeneration with the iron in the steel alloy which comprises constructing those portions of the apparatus exposed to the hot gases during regeneration of steel containing from 24 to 26% chromium, 19 to 21% nickel, 0.2 to 1.8% silver and the balance iron and small amounts of carbon and other impurities which do not interfere with the effect of the silver on the steel.

ROBERT P. RUSSELL.